# EUROPEAN PATENT SPECIFICATION

(11) **EP 2 177 639 B1**
(45) Date of publication and mention of the grant of the patent: **04.03.2020**
(21) Application number: 08791644.1
(22) Date of filing: 25.07.2008
(51) Int. Cl.: C22C 29/04, B23B 27/14, C22C 1/05, B22F 7/06

(54) **TITANIUM-BASE CERMET, COATED CERMET, AND CUTTING TOOL**
CERMET AUF TITANBASIS, BESCHICHTETER CERMET UND SCHNEIDWERKZEUG
CERMET À BASE DE TITANE, CERMET ENROBÉ ET OUTIL TRANCHANT

(30) Priority: 27.07.2007 JP 2007195909; 27.07.2007 JP 2007195910; 28.11.2007 JP 2007306887
(43) Date of publication of application: 21.04.2010
(73) Proprietor: KYOCERA CORPORATION, Kyoto-shi, Kyoto (JP)
(72) Inventor: TOKUNAGA, Takashi, Satsumasendai-shi Kagoshima 895-0292 (JP); KINOSHITA, Hideyoshi, Satsumasendai-shi Kagoshima 895-0292 (JP)
(74) Representative: Viering, Jentschura & Partner mbB Patent- und Rechtsanwälte
(86) International application number: PCT/JP2008/063400
(87) International publication number: WO 2009/017053

(56) References cited:
- EP-A1- 1 462 534
- JP-A- 2004 115 881
- JP-A- 2004 292 905
- US-B1- 6 190 762

## Description

### TECHNICAL FIELD

The present invention relates to a titanium (Ti)-based cermet, a coated cermet, and a cutting tool, particularly to a cutting tool whose cutting edge has enhanced wear resistance.

### BACKGROUND ART

Sintered alloys such as cemented carbides composed mainly of WC, and Ti-based cermet composed mainly of Ti are currently widely used as members requiring wear resistance and sliding properties, as well as fracture resistance, such as cutting tools, wear-resistant members and sliding members. Developments of novel compositions for improving performance of these sintered alloys have been continued.

For example, patent document 1 discloses the technique of forming cemented carbide or a cermet by reaction sintering using microwaves, and describes that Mn or Al is added in the proportion of 5% by mass or less into a metal binder phase such as Co.

Patent document 2 discloses the gradient composition sintered alloy made by adding 0.1 to 10% by mass of a specific metal element such as Mn, in addition to a hard phase composed mainly of carbides or nitrides of metals selected from Group 4, Group 5 and Group 6 metals of the periodic table, and mutual solid solutions of these, and 1 to 40% by mass of an iron-group metal. Ti-based cermets made by adding Mn are described in Samples No. 17 and No. 20 in Table 6. Table 8 indicates that the concentration of the Mn and the concentration of the binder phase in Sample No. 17 and No. 20 are increased in the interior of the cermet than the surface thereof.
Patent document 1: Japanese Unexamined Patent Publication No. 2000-503344
Patent document 2: Japanese Unexamined Patent Publication No. 2004-292905

### DISCLOSURE OF THE INVENTION

### PROBLEMS TO BE SOLVED BY THE INVENTION

However, there is a limit to the improvements in the hardness and toughness of the cermet with the method in which Mn is added and then microwave sintered, as described in the patent document 1. Even in the gradient composition having the increased Mn concentration and the increased binder phase concentration in the interior of the sintered body, as described in the patent document 2, there is the problem that the effect in improving the hardness of the cermet surface remains insufficient, and the finish-machined surface of a work material becomes rough due to the welding of the work material onto the cutting edge, thus causing abnormal wear or fracture.

Therefore, the cutting tool of the present invention has been made to solve the above problems, and aims to enhance the wear resistance and welding resistance of the Ti-based cermet.

### MEANS FOR SOLVING THE PROBLEMS

The present invention provides a Ti-based cermet according to claim 1. A further advantageous embodiment of the Ti-based cermet according to the present invention is disclosed in dependent claim 2.

The present invention further provides a method of manufacturing a Ti-based cermet according to claim 3.

The present invention further provides a coated cermet according to claim 4. Further advantageous embodiments of the coated cermet according to the present invention are disclosed in dependent claims 5-10.

The present invention further provides a cutting tool according to claim 11. A further advantageous embodiment of the cutting tool according to the present invention is disclosed in dependent claim 12.

### EFFECT OF THE INVENTION

In accordance with the Ti-based cermet of the invention, 0.1 to 0.5% by mass of Mn is contained, and the surface region, in which the second hard phase whose content percentage is not less than 90% by area is observed, is formed in the surface of the cermet. This increases the toughness of the cermet as a whole, and enhances the hardness in the surface of the cermet, thereby improving wear resistance and also enhancing

The coated cermet of the invention is produced by using the above Ti-based cermet as a substrate, and coating a surface of the substrate with a coating layer. The content ratio of the binder phase in the surface region of the substrate is not more than 3% by mass, and the coating layer is formed by chemical vapor deposition.

The cutting tool of the invention is composed of the above Ti-based cermet or the above coated cermet, and a cutting edge is formed along a cross ridge part between a rake face and a flank face. In the residual stress measured by 2D method in the rake face which is exerted in a σ₁₁ direction (a direction to connect between the center of the rake face and the center of the cutting edge nearmost the measured point), the second hard phase is preferably subjected to compressive stress of not less than 150 MPa (σ₁₁ ≤ -150 MPa).

### EFFECT OF THE INVENTION

In accordance with the Ti-based cermet of the invention, 0.1 to 0.5% by mass of Mn is contained, and the surface region, in which the second hard phase whose content percentage is not less than 90% by area is observed, is formed in the surface of the cermet. This increases the toughness of the cermet as a whole, and enhances the hardness in the surface of the cermet, thereby improving wear resistance and also enhancing welding resistance.

### PREFERRED EMBODIMENTS FOR CARRYING OUT THE INVENTION

### <Ti-based Cermet>

An example of the Ti-based cermet of the invention will now be described based on the scanning electron microscope (SEM) photograph of the cross-section of the important parts including the surface region of the Ti-based cermet as shown in Fig. 1.

The Ti-based cermet (hereinafter referred to simply as "cermet") 1 in Fig. 1 is composed of at least one kind of element selected from Co and Ni; and one or more kinds of substances selected from carbides, nitrides, and carbonitrides of one or more kinds of metals selected from Group 4, Group 5, and Group 6 metals of the periodic table, composed mainly of Ti; and 0.1 to 0.5% by mass of Mn.

As shown in Fig. 1, in the scanning electron microscope (SEM) photograph of an arbitrary cross-section, a surface region 5 is formed in which a hard phase 2 whose interior comprises a black first hard phase 2a and a grayish white second hard phase 2b, and a binder phase 3 composed mainly of at least one kind of elements selected from Co and Ni are observed, and the second hard phase 2b whose content percentage is not less than 90% by area is observed in a surface part.

This increases the toughness of the cermet as a whole, and enhances the hardness in the surface of the cermet, thereby improving wear resistance and also enhancing welding resistance.

In the scanning electron microscope (SEM) photograph of the cross-sectional structure of the cermet 1 as shown in Fig. 1, the first hard phase 2a is observed as black particles, and the second hard phase 2b is observed as grayish white particles, or particles having a core-containing structure in which a grayish white peripheral part exists around a white core part. That is, the first hard phase 2a has a higher content ratio of a light element than the second hard phase 2b, and hence looks black. Although the first hard phase 2a corresponds to the black particles composed of TiCN, it may contain Co or Ni. Alternatively, other core-containing structure may be employed in which the grayish white second hard phase 2b exists as a peripheral part in the outer periphery of the first hard phase 2a. On the other hand, the binder phase 3 is observed as a white region, and Co and Ni constituting the binder phase 3 can be confirmed by energy dispersive spectroscopy (EMPA) annexed to the scanning electron microscope (SEM).

Unless not less than 0.1% by mass of Mn is contained in the cermet 1, the toughness of the cermet 1 is lowered. Conversely, if more than 0.5% by mass of Mn is contained in the cermet 1, the hardness of the cermet 1 is remarkably lowered. The suitable content of Mn is 0.2 to 0.5% by mass.

In the absence of the surface region 5 in the surface of the cermet 1, the hardness in the surface of the cermet 1 cannot be enhanced, thus leading to insufficient wear resistance of the cermet 1. If the percentage of presence of the second hard phase 2b in the surface region 5 is less than 90% by area, the wear resistance and welding resistance in the surface of the cermet 1 become insufficient. The suitable thickness of the surface region 5 is 0.8 to 3 µm. The preferable percentage of area Bₛ of the second hard phase 2b in the surface region 5 is 93 to 97% by area, in the interest of adhesion with respect to a coating layer 13.

Like the scanning electron microscope (SEM) photograph of the cross-section in the vicinity of the surface of the cermet 1 as shown in Fig. 1, the average particle diameter d₁ₛ of the second hard phase 2b is preferably 0.5 to 3.0 µm, particularly 1.0 to 2.0 µm. The ratio (Cₛ/Cᵢ) of the content ratio Cₛ of the binder phase 3 in the surface region 5 to the content ratio Cᵢ of the binder phase 3 in the interior is preferably 0.01 to 0.1, with the view of enhancing the wear resistance in the surface of the cermet 1 and enhancing the welding resistance in the surface of the cermet 1.

When the cross-sectional structure in the interior of the cermet 1 is further observed, the average particle diameter of the second hard phase 2b is larger than the average particle diameter of the first hard phase 2a, preferably the ratio (bᵢ/aᵢ) of aᵢ and bᵢ is 2 to 8, where aᵢ is the average particle diameter of the first hard phase 2a in the interior, and bᵢ is the average particle diameter of the second hard phase 2b in the interior, in the point that the second hard phase 2b effectively contributes to thermal propagation thereby to improve the thermal conductivity of the cermet 1 and improve the thermal shock resistance of the cermet 1. The suitable ratio (bᵢ/aᵢ) of aᵢ and bᵢ is 3.5 to 7, with the view of maintaining the fracture resistance of the cermet 1.

In the present invention, the particle diameter of the hard phase 2 is measured according to the method of measuring the average particle diameter of cemented carbide as prescribed in CIS-019D-2005. Specifically, when the hard phase 2 has the core-containing structure, the region extending up to the outer edge of the peripheral part including the core part and the peripheral part is regarded as a single hard phase, and the particle diameter thereof is measured. When observing the cross-sectional structure in the interior of the cermet 1 of the invention, the region extending in a depth of not less than 1000 µm from the surface of the cermet 1 is observed.

Further in the cross-sectional structure of the interior of the cermet 1, the average area of the second hard phase 2b is larger than the average area of the first hard phase 2a, preferably the ratio (Bᵢ/Aᵢ) of A₁ and B₁ is 1.5 to 5, where Aᵢ is the average area occupied by the first hard phase 2a, and Bᵢ is the average area occupied by the second hard phase 2b, with respect to the entirety of the hard phase 2 in the interior, in the point that the second hard phase 2b more effectively contributes to thermal propagation thereby to improve the thermal conductivity of the cermet 1 and improve the thermal shock resistance of the cermet 1.

In the interior of the cermet 1, the total content ratio of nitrides or carbonitrides of Group 4, Group 5 and Group 6 metals of the periodic table, each of which constitutes the hard phase 2 and is composed mainly of Ti, is preferably 70 to 96% by mass, particularly 85 to 96% by mass, with the view of improving wear resistance. On the other hand, the content ratio of the binder phase 3 is preferably 4 to 30% by mass, particularly 4 to 15% by mass. This achieves excellent balance between the hardness and toughness of the cermet 1. The binder phase 3 preferably contains not less than 65% by mass of Co with respect to the total amount of iron-family metals with the view of enhancing the thermal shock resistance of a cutting tool. In order to maintain satisfactory sintering properties of the cermet 1 so that the baked surface of the cermet 1 becomes a smooth surface, it is preferable to contain 5 to 50% by mass of Ni, particularly 10 to 35% by mass of Ni with respect to the total amount of iron-family metals.

### <Coated Cermet>

A coating layer can be formed on the surface of the above cermet 1. An example thereof will now be described based on Fig. 2, wherein (a) is a scanning electron microscope (SEM) photograph of important parts in a cross-section including a surface region of a coated cermet 10, and (b) is a scanning electron microscope (SEM) photograph of important parts of a ground surface before forming the coating layer of the coated cermet 10.

The coated cermet 10 of Fig. 2(a) has the structure that the surface of a substrate 12 composed of the above cermet 1 is coated with the coating layer 13.

In the present invention, as shown in Fig. 2, the coating layer 13 formed by chemical vapor deposition (CVD) method can also be formed. That is, conventional coated cermets generally employ physical vapor deposition (PVD) method carried out with the substrate heated to approximately 500°C. This is because if used CVD method that is carried out with a substrate heated to high temperatures of 700°C and above, the coating layer may cause partially abnormal particle growth and change into a needle shape due to Ni or Fe used as the binder phase of the Ti-based cermet, and the strength of the coating layer may be lowered, causing chipping or fracture. However, the cermet 1 as the substrate 12 of the invention is adapted to reduce the existence of Ni in the surface of the substrate 12, and hence the coating layer 13 does not cause any abnormal particle growth. It is also capable of preventing the hardness deterioration of the coating layer 13 due to a large amount of diffusion of the binder phase 3 into the coating layer 13. Consequently, the coating layer 13 has high hardness and high strength characteristics. Additionally, when the surface region 5 and the coating layer 13 are similar to each other in structural components and crystal structure, there is a slight difference in thermal expansion coefficients between the two, and hence separation due to thermal stress does not occur in the interface between the substrate 12 and the coating layer 13.

The surface region 5, in which the content ratio of the binder phase 3 is not more than 3% by mass, exists in the region extending 0.1 to 5 µm from the surface of the substrate 12, as shown in Fig. 2(b). The coating layer 13 is formed by CVD method. This enhances the adhesion of the coating layer 13 with respect to the substrate 12 without deteriorating the hardness of the coating layer 13, thereby enhancing the fracture resistance in the surface of the coated cermet 10.

That is, in the absence of the surface region 5 in the surface of the substrate 12, Ni exists in the surface of the substrate 12, and the coating layer 13 to be formed in the surface causes abnormal particle growth, thus deteriorating both hardness and toughness.

In the substrate 12, the thickness of the surface region 5 is preferably 0.8 to 3 µm, with the view of maintaining the shock resistance of the coated cermet 10. The percentage of area Bₛ of the second hard phase 2b in the surface region 5 is preferably 70 to 100% by area to the entirety of the hard phase 2, with the view of enhancing the adhesion with respect to the coating layer 13.

Preferably, a binder phase-rich region 8 exists in a region extending 1 to 10 µm from immediately below the surface region 5, at 1.1 to 2.0 in terms of the ratio (A/B) of A to B, where A is the content ratio of the binder phase 3, and B is the content ratio of the binder phase 3 in the interior of the substrate 12. Thus, even if the coating layer 13 is subjected to shock, the binder phase-rich region 8 relaxes the shock and reduces chipping or fracture in the coating layer 13.

In the coating layer 13, if the content of the binder phase 3 in the region extending up to 0.1 to 5 µm from the surface of the substrate 12 is larger than 3% by mass, the ingredients of the binder phase 3 diffuse into the coating layer 13, thus deteriorating the hardness of the coating layer 13.

In order to maintain satisfactory sintering properties for achieving a smooth burned surface of the substrate 12, and also enhance the thermal shock resistance of the substrate 12, it is preferable for the binder phase 3 that the content ratio of Ni in the interior of the substrate is 0.1 to 0.5 in terms of Ni/(Ni+Co) ratio.

When the content ratio of N in the surface region 5 is larger than that in the interior of the sintered body, the surface region 5 has excellent toughness characteristic. Therefore, when the coating layer 13 having a higher hardness than the surface region 5 is formed immediately above the surface region 5, the high-hard and brittle coating layer 13 causes neither chipping nor separation even under shock exerted during cutting or the like, thereby achieving satisfactory wear resistance and fracture resistance. The distribution of the content ratio of N can be compared by X-ray photoelectron spectroscopic analysis in a depth direction from the surface of the cermet 1 toward the interior thereof.

On the other hand, the coating layer 13 is composed of a columnar crystal extending vertically with respect to the surface of the substrate 12. The coating layer 13 preferably includes a columnar crystal coating layer in which the columnar crystal has an average crystal width of 0.1 to 1 µm, in the interest of high fracture resistance and excellent wear resistance of the coating layer 13. As the columnar crystal coating layer, a TiCN layer is suitable in the interest of easy manufacture of the above-mentioned structure. In this case, the coating layer is capable of producing the above effect irrespective of whether the coating layer is a single columnar crystal coating layer, or a multilayer structure made up of one or more columnar crystal coating layers and other layer. The TiCN layer composed of the TiCN columnar crystal included in the coating layer 13 preferably has its strongest peak in (422) plane in an X-ray diffraction measurement, in the interest of high wear resistance of the coating layer 13 and excellent adhesion with respect to the substrate 12.

### <Cutting Tool>

An example of the cutting tool of the invention will now be described with reference to Figs. 3(a) and 3(b), which are schematic perspective views thereof.

Referring to Fig. 3, the cutting tool 20 of the invention is constructed to have a rake face 21 on the main surface thereof, a flank face 22 on the side surface thereof, and cutting edges 23 (23a to 23d) along a cross ridge line between the rake face 21 and the flank face 22. As shown in Fig. 3, a recessed part 25 including a breaker 24 is formed in the rake face 21. A screw hole 26 for mounting the cutting tool 20 onto a holder (not shown) is formed at the center of the rake face 21.

The method of machining a work material includes the following three steps. In the first step, the cutting tool 20 made of the cermet 1 or the coated cermet 10 and provided with the cutting edges 23 is prepared. In the next step, the cutting edge 23 of the cutting tool 20 is brought into contact with the work material. In the last step, the work material is subjected to cutting by using the cutting tool 20.

According to the present invention, in the residual stress exerted in the σ₁₁ direction (a direction to connect between the center of the rake face 21 and the cutting edge 23a nearmost the measured point) measured by 2D method in a portion P other than the recessed part of the rake face 21, the second hard phase 2b is preferably subjected to compressive stress of not less than 150 MPa (σ₁₁ ≤ -150 MPa). This improves the fracture resistance in the cutting edges 23.

### <Manufacturing Method>

An example of the method of manufacturing the above cermet will be described below.

Firstly, a mixed powder is prepared by mixing TiCN powder having an average particle diameter of 0.1 to 2 µm, preferably 0.2 to 1.2 µm, one kind of powder selected from carbide powder, nitride powder and carbonitride powder of the above-mentioned other metal having an average particle diameter of 0.1 to 2 µm, Co powder or Ni powder, metal Mn powder or Mn compound powder having an average particle diameter of 0.5 to 10 µm, wherein a total amount in terms of Mn is 0.2 to 3.0% by mass.

Subsequently, a binder is added to the mixed powder and formed into a predetermined shape by any known forming method such as press forming, extrusion forming, injection forming, or the like.

According to the present invention, the cermet having the predetermined structure described above can be manufactured by performing sintering steps under the following conditions. The sintering conditions are as follows: (a) Temperature is increased under vacuum from room temperature to 1200°C; (b) The temperature is increased under vacuum at a temperature rising rate r₁ of 0.1 to 2°C/min from 1200°C to a sintering temperature T₁ of 1330 to 1380 °C; (c) The temperature is increased in an inert gas atmosphere of 30 to 2000 Pa at a temperature rising rate r₂ of 4 to 15°C/min from the sintering temperature T₁ to a sintering temperature T₂ of 1450 to 1600°C; (d) The sintering temperature T₂ is retained for 0.5 to 2 hours in an inert gas atmosphere of 30 to 2000 Pa; and (e) The temperature is decreased.

That is, among the above sintering conditions, if the sintering atmosphere in the step (b) is an inert gas atmosphere instead of under vacuum, the volatilization of Mn is reduced, and the content of Mn in the cermet after sintering cannot be controlled, and the above surface region is not formed. The surface region is also not formed if the temperature rising rate in the step (b) is higher than 2°C/min. If the atmosphere in the step (c) is under vacuum or an inert gas atmosphere of less than 30 Pa, more than 0.5% by mass of Mn remains in the interior of the cermet 1, and the surface region is not formed. Conversely, if it is a high inert gas atmosphere exceeding 2000 Pa, the surface region is not formed. If the sintering temperature T₂ in the step (d) is below 1450°C, the surface region is not formed. If the sintering temperature T₂ exceeds 1600°C, the surface region of not less than 5 µm is formed, resulting in poor toughness.

The surface region 5 having high hardness and high welding resistance is achieved by performing the temperature decreasing step (e) in a vacuum atmosphere. If the temperature decreasing step (e) is performed in an inert gas atmosphere, the content ratio of N in the surface region 5 becomes larger than that in the interior of the cermet 1, thereby forming the surface region having high toughness.

Preferably, a coating layer is coated onto the surface of the substrate composed of the above cermet at 800 to 1100°C by CVD method. Specific film forming conditions are as follows. Firstly, a titanium nitride (TiN) layer is formed by preparing in a CVD furnace a mixed gas composed of, for example, 0.1 to 10% by volume of titanium chloride (TiCl₄), 10 to 60% by volume of nitrogen (N₂) gas, and the rest that is hydrogen (H₂) gas, and by admitting the mixed gas into a reaction chamber, followed by controlling the inside of the chamber in the range of 800 to 1100°C and 50 to 85 kPa.

Subsequently, with so-called MT-CVD method, a titanium carbonitride (TiCN) layer is formed on the titanium nitride (TiN) layer by admitting a mixed gas prepared so that titanium chloride (TiCl₄) is 0.5 to 5.0% by volume, acetonitrile (CH₃CN) is 0.3 to 1.5% by volume, nitrogen (N₂) is 10 to 40% by volume, and the rest is hydrogen (H₂), at a reaction temperature of 800 to 900°C.

With regard to the above film forming conditions, by adjusting the proportion of acetonitrile gas in the gas to the above-mentioned range, the structure of the titanium carbonitride (TiCN) in the titanium carbonitride (TiCN) layer can be surely grown within the above-mentioned range. The titanium carbonitride (TiCN) layer composed of the columnar crystal having an average crystal width of 0.1 to 1 µm can be formed by setting the film forming temperature to 800°C to 850°C, and by controlling, in the titanium carbonitride (TiCN) crystal growth step in the early period of forming the titanium carbonitride (TiCN) layer, the proportion V_{A} of the acetonitrile (CH₃CN) gas in the range of 0.3 to 1.5% by volume, and also controlling the ratio (V_{A}/V_{H}) of the proportion V_{H} of the hydrogen gas (H₂) as carrier gas and the proportion V_{A} of the acetonitrile (CH₃CN) gas at a low concentration of not more than 0.03. The TiCN layer has a film thickness of not less than 2 µm, and (422) peak becomes the strongest in an XRD diffraction.

Next, a titanium oxycarbonitride (TiCNO) layer is formed by preparing and admitting a mixed gas composed of 0.1 to 3% by volume of titanium chloride (TiCl₄) gas, 0.1 to 10% by volume of methane (CH₄) gas, 0.01 to 5% by volume of carbon dioxide (CO₂) gas, 0.1 to 60% by volume of nitrogen (N₂) gas, and the rest that is hydrogen (H₂) gas, into the reaction chamber, and by controlling the conditions within the chamber in the range of 800 to 1100°C and 5 to 30 kPa.

Subsequently, an aluminum oxide (Al₂O₂) layer is formed by using a mixed gas composed of 3 to 20% by volume of aluminum chloride (AlCl₃) gas, 0.5 to 3.5% by volume of hydrogen chloride (HCl) gas, 0.01 to 5% by volume of carbon dioxide (CO₂) gas, 0 to 0.01% by volume of hydrogen sulfide (H₂S) gas, and the rest that is hydrogen (H₂) gas, and by controlling in the range of 900 to 1100°C and 5 to 10 kPa.

Further, a titanium nitride (TiN) layer is formed by preparing and admitting a mixed gas composed of 0.1 to 10% by volume of titanium chloride (TiCl₄) gas, 10 to 60% by volume of nitrogen (N₂) gas, and the rest that is hydrogen (H₂) gas, into the reaction chamber, and by controlling the conditions within the chamber in the range of 800 to 1100°C and 50 to 85 kPa.

Thereafter, as required, a predetermined portion of the surface of the formed coating layer 8 is subjected to mechanical grinding by means of brush, elastic grinding, or blast method. This grinding adjusts the residual stress generated during film formations and remaining in the coating layer.

### Example 1

A mixed powder was prepared by blending, in the proportions shown in Table 1, TiCN powder having an average particle diameter of 0.6 µm, WC powder having an average particle diameter of 1.1 µm, TiN powder having an average particle diameter of 1.5 µm, TaC powder having an average particle diameter of 2 µm, MoC powder having an average particle diameter of 1.5 µm, NbC powder having an average particle diameter of 1.5 µm, ZrC powder having an average particle diameter of 1.8 µm, VC powder having an average particle diameter of 1.0 µm, Ni powder having an average particle diameter of 2.4 µm, Co powder having an average particle diameter of 1.9 µm, and MnCO₃ powder having an average particle diameter of 5.0 µm. These average particle diameters (d₅₀ values) were measured by microtrack method. The mixed powder was then wet mixed while adding isopropyl alcohol (IPA), and then 3% by mass of paraffin was added and mixed together by using a ball mill and carbide balls made of stainless steel. Subsequently, this mixed powder was press-formed into a throw-away tip tool shape of CNMG120408 at an applied pressure of 200 MPa. Thereafter, throw-away tips made of the cermets of Samples Nos. 1 to 11, respectively, were obtained through the following steps: (a) Temperature was increased under vacuum from room temperature to 1200°C at 10°C/min; (b) The temperature was increased in the sintering atmosphere and at the temperature rising rate r₁ (°C/min) shown in Table 2, from 1200°C to the sintering temperature T₁ shown in Table 2; (c) The temperature was increased in the sintering atmosphere shown in Table 2, at the temperature rising rate r₂ (°C/min) shown in Table 2, from the sintering temperature T₁ to the sintering temperature T₂ shown in Table 2; (d) Sintering was carried out in the sintering atmosphere at the sintering temperature and the sintering time shown in Table 2; and (e) The temperature was decreased in the sintering atmosphere shown in Table 2.

**[Table 1]**

| Sample No. | Material composition (% by mass) | | | | | | | | | | |
|---|---|---|---|---|---|---|---|---|---|---|---|
| | TiCN | WC | TiN | TaC | MoC | NbC | ZrC | VC | Ni | Co | MnCO₃ |
| 1 | 51.5 | 17 | 10 | 3 | 0 | 10 | 1 | 1 | 2 | 3 | 1.5 |
| 2 | 63.5 | 10 | 5 | 1 | 1 | 8 | 2 | 1 | 2 | 6 | 0.5 |
| 3 | 57 | 15 | 8 | 0 | 1 | 5 | 2 | 1 | 3 | 6 | 2 |
| 4 | 58 | 12 | 7 | 0 | 2 | 8 | 1 | 2 | 2 | 7 | 1 |
| 5 | 53.5 | 10 | 12 | 3 | 0 | 6 | 1 | 1 | 4 | 7 | 2.5 |
| 6 | 54.5 | 15 | 3 | 0 | 0 | 9 | 1 | 2 | 2 | 12 | 1.5 |
| 7 | 58 | 13 | 7 | 2 | 0 | 10 | 1 | 1 | 2 | 5 | 1 |
| * 8 | 49 | 14 | 12 | 3 | 0 | 8 | 2 | 2 | 4 | 6 | - |
| * 9 | 49 | 14 | 12 | 3 | 0 | 8 | 2 | 2 | 4 | 6 | 1 |
| * 10 | 48 | 17 | 10 | 1 | 1 | 9 | 2 | 1 | 3 | 7 | 1 |
| * 11 | 48 | 17 | 10 | 1 | 1 | 9 | 2 | 1 | 3 | 7 | 1 |

| | | | | | | | | | | | |
|---|---|---|---|---|---|---|---|---|---|---|---|
| The samples marked "*" are out of the scope of the present invention. | | | | | | | | | | | |

**[Table 2]**

| Sample No. | Sintering condition | | | | | | | | | | | | |
|---|---|---|---|---|---|---|---|---|---|---|---|---|---|
| | Step (b) | | | | Step (c) | | | | Step (d) | | | Step (e) | |
| | Temperature rising rate r₁ (°C/min) | Sintering temperature T₁ (°C) | Sintering atmosphere | | Temperature rising rate r₂ (°C/min) | Sintering temperature T₂ (°C) | Sintering atmosphere | | Sintering time (hr) | Sintering atmosphere | | Sintering atmosphere | |
| 1 | 1.5 | 1350 | Vacuum | | 5 | 1550 | N₂ | 500Pa | 1.5 | N₂ | 500Pa | Vacuum | |
| 2 | 0.7 | 1350 | Vacuum | | 10 | 1525 | Ar | 80Pa | 1 | Ar | 80Pa | Vacuum | |
| 3 | 0.5 | 1350 | Vacuum | | 7 | 1600 | N₂ | 800Pa | 0.5 | N₂ | 800Pa | Vacuum | |
| 4 | 0.7 | 1360 | Vacuum | | 8 | 1575 | N₂ | 1000Pa | 1 | N₂ | 1000Pa | Vacuum | |
| 5 | 1 | 1380 | Vacuum | | 4 | 1450 | N₂ | 300Pa | 2 | N₂ | 300Pa | Vacuum | |
| 6 | 0.3 | 1330 | Vacuum | | 15 | 1550 | N₂ | 700Pa | 1 | N₂ | 700Pa | Vacuum | |
| 7 | 0.7 | 1340 | Vacuum | | 10 | 1575 | He | 1000Pa | 1 | He | 1000Pa | Vacuum | |
| * 8 | 1 | 1350 | Vacuum | | 10 | 1550 | He | 1200Pa | 1 | He | 1200Pa | He | 1200Pa |
| * 9 | 5 | 1350 | Vacuum | | 5 | 1550 | He | 1200Pa | 1 | He | 1200Pa | He | 1200Pa |
| * 10 | 1.0 | 1350 | N₂ | 800Pa | 2 | 1650 | N₂ | 800Pa | 1 | N₂ | 800Pa | N₂ | 800Pa |
| * 11 | 1.0 | 1350 | N₂ | 800Pa | 8 | 1550 | Vacuum | | 1 | Vacuum | | Vacuum | |

| | | | | | | | | | | | | | |
|---|---|---|---|---|---|---|---|---|---|---|---|---|---|
| The samples marked "*" are out of the scope of the present invention. | | | | | | | | | | | | | |

Each of the obtained cermets was subjected to a scanning electron microscope (SEM) observation, and an image analysis was performed using commercially available image analysis software onto arbitrary five points in the surface and the interior thereof, respectively, at a region of 8 µm × 8 µm in a photograph taken at 10000 magnification. Then, it was confirmed whether or not the surface region existed by observing the existing states of the hard phase and the binder phase, and the structure states in the interior and the surface. In all the individual samples, it was confirmed that the binder phase was composed mainly of Co and Ni, based on the energy dispersive spectroscopic analysis (EMPA) annexed to the scanning electron microscope (SEM). Subsequently, the average particle diameter of the hard phase in the above region of each sample was measured, and the ratio thereof was calculated. The results were shown in Table 3. Further, the content ratio of the metal Mn ingredient in the interior of the cermet substrate of each sample was determined by ICP analysis. The results were shown in Table 3.

Next, these cutting tools made of the obtained cermets were subjected to a cutting test under the following cutting conditions. The results were also shown in Table 3.

| | |
|---|---|
| Work material: | SCM435 |
| Cutting speed: | 200m/min |
| Feed rate: | 0.20mm/rev |
| Depth of cut: | 1.0mm |
| Cutting state: | Wet (using water-soluble cutting fluid) |
| Evaluation method: | Time (min) elapsed until the amount of wear reached 0.2mm |

**[Table 3]**

| Sample No. | Interior | | | | | | | Mn ratio (% by mass) | Surface region | | | | | Cutting performance⁹⁾ |
|---|---|---|---|---|---|---|---|---|---|---|---|---|---|---|
| | dᵢ¹⁾ | aᵢ²⁾ | bᵢ³⁾ | bᵢ/aᵢ | Aᵢ⁴⁾ | Bᵢ⁵⁾ | Bᵢ/Aᵢ | | bₛ⁶⁾ | bₛ/bᵢ | Bₛ⁷⁾ | cₛ/cᵢ⁸⁾ | Thickness (*µ*m) | |
| 1 | 0.44 | 0.40 | 1.26 | 3.15 | 26 | 74 | 2.85 | 0.25 | 1.85 | 1.47 | 93 | 0.05 | 2.1 | 53 |
| 2 | 0.50 | 0.26 | 0.90 | 3.46 | 38 | 62 | 1.63 | 0.12 | 1.20 | 1.33 | 92 | 0.08 | 0.8 | 46 |
| 3 | 0.45 | 0.37 | 1.38 | 3.73 | 25 | 75 | 3.00 | 0.30 | 2.13 | 1.54 | 91 | 0.10 | 3.9 | 55 |
| 4 | 0.50 | 0.21 | 1.05 | 5.00 | 37 | 63 | 1.70 | 0.20 | 1.58 | 1.50 | 94 | 0.07 | 2.8 | 57 |
| 5 | 0.49 | 0.18 | 0.95 | 5.28 | 40 | 60 | 1.50 | 0.40 | 1.27 | 1.34 | 96 | 0.02 | 2.5 | 50 |
| 6 | 0.45 | 0.35 | 1.26 | 3.60 | 27 | 73 | 2.70 | 0.15 | 1.95 | 1.55 | 91 | 0.08 | 4.5 | 52 |
| 7 | 0.40 | 0.49 | 1.75 | 3.57 | 18 | 82 | 4.56 | 0.12 | 2.11 | 1.21 | 93 | 0.03 | 1.5 | 48 |
| * 8 | 0.41 | 0.28 | 1.21 | 4.32 | 27 | 73 | 2.70 | <0.05 | Absence | | | | | 32 |
| * 9 | 0.57 | 0.28 | 1.21 | 4.32 | 35 | 65 | 1.86 | 1.00 | Absence | | | | | 35 |
| * 10 | 0.34 | 0.37 | 1.42 | 3.84 | 19 | 81 | 4.26 | 0.07 | 2.21 | 1.56 | 91 | 0.1 | 8 | 39 |
| * 11 | 0.33 | 0.35 | 1.25 | 3.57 | 21 | 79 | 3.76 | 0.13 | Absence | | | | | 37 |

| | | | | | | | | | | | | | | |
|---|---|---|---|---|---|---|---|---|---|---|---|---|---|---|
| The samples marked "*" are out of the scope of the present invention. 1) dᵢ: Average particle diameter (*µ*m) of whole hard phase in interior 2) aᵢ: Average particle diameter (*µ*m) of first hard phase in interior 3) bᵢ: Average particle diameter (*µ*m) of second hard phase in interior 4) Aᵢ: Percentage of area (% by area) of first hard phase in interior 5) Bᵢ: Percentage of area (% by area) of second hard phase in interior 6) bₛ: Average particle diameter (*µ*m) of second hard phase in surface region 7) Bₛ: Percentage of area (% by area) of second hard phase in surface region 8) cₛ/cᵢ: Content ratio cₛ of binder phase in surface region / content ratio cᵢ of binder phase in interior 9) Cutting performance: Time (min) elapsed until amount of wear reached 0.2mm | | | | | | | | | | | | | | |

The followings will be noted from Tables 1 to 3. That is, in Sample No. 8 without Mn addition, the surface region was not formed and wear occurred early. In Sample No. 10 in which the sintering temperature was higher than 1600°C and the content of Mn is less than 0.1% by mass, the wear resistance thereof was deteriorated due to the occurrence of chipping. Also in Sample No. 9 in which the content of Mn exceeded 0.5% by mass, the wear resistance thereof was poor. In Sample No. 11 in which the surface region was not formed due to the mismatched sintering conditions, the wear resistance thereof was lowered.

On the contrary, all Samples Nos. 1 to 7, which were the cermets having the structures within the scope of the invention, exhibited excellent wear resistance and satisfactory wear resistance, thereby achieving a long tool life.

The residual stress in the rake face of each of Samples Nos. 4, 7 and 11 was measured by 2D method (an X-ray diffraction apparatus manufactured by Bruker AXS Inc., D8 DISCOVER with GADDS Super Speed, Ray source: CuK_{α}, Collimater diameter: 0.3mmΦ, Measured diffraction line: TiN (422) plane). In the residual stress exerted in the σ₁₁ direction (the direction to connect between the center of the rake face and the center of the cutting edge nearmost the measured point), the individual second hard phases were subjected to compressive stress of 250 MPa (σ₁₁ = -250 MPa), 150 MPa (σ₁₁ = -150 MPa), 100 MPa (σ₁₁ = -100 MPa), respectively.

### Example 2

Cermets were manufactured under the same manufacturing conditions as in the throw-away tips made of the cermets of Samples Nos. 1 to 11 in Example 1, except for changing the atmosphere in the temperature decreasing step (e) into the atmospheres shown in Table 4. Similarly to Example 1, the structures of the obtained cermets were observed and the results thereof were shown in Table 5. In each of these cermets, the content of N in the interior of the cermet and that in the surface region thereof were compared by performing the X-ray photoelectron spectroscopic analysis in a depth direction from the surface of the sintered body to the interior thereof. Then, the ratio of the content of N in the surface region to the content of N in the interior was shown in Table 6. Thereafter, throw-away tips of Samples Nos. 12 to 18 were obtained by forming the coating layers of Table 6 on these cermets, respectively. The obtained throw-away tips made of the cermets were subjected to a cutting test under the same cutting conditions as Example 1. The results were also shown in Table 6.

**[Table 4]**

| Sample No. | Material composition No. for substrates | Sintering condition | | | | | | | | | | | |
|---|---|---|---|---|---|---|---|---|---|---|---|---|---|
| | | Step (b) | | | Step (c) | | | | Step (d) | | | Step (e) | |
| | | Temperature rising rate r₁ (°C/min) | Sintering temperature T₁ (°C) | Sintering atmosphere | Temperature rising rate r₂ (°C/min) | Sintering temperature T₂ (°C) | Sintering atmosphere | | Sintering time (hr) | Sintering atmosphere | | Sintering atmosphere | |
| 12 | 1 | 1.5 | 1350 | Vacuum | 5 | 1550 | N₂ | 500Pa | 1 | N₂ | 500Pa | N₂ | 100Pa |
| 13 | 2 | 0.7 | 1350 | Vacuum | 10 | 1525 | Ar | 80Pa | 0.5 | Ar | 80Pa | N₂ | 500Pa |
| 14 | 3 | 0.5 | 1350 | Vacuum | 7 | 1600 | N₂ | 800Pa | 1.5 | N₂ | 800Pa | N₂ | 1000Pa |
| 15 | 4 | 0.7 | 1360 | Vacuum | 8 | 1575 | N₂ | 1000Pa | 1 | N₂ | 1000Pa | N₂ | 1500Pa |
| 16 | 5 | 1 | 1380 | Vacuum | 4 | 1450 | N₂ | 600Pa | 2 | N₂ | 600Pa | N₂ | 900Pa |
| 17 | 6 | 0.3 | 1330 | Vacuum | 15 | 1550 | N₂ | 700Pa | 1 | N₂ | 700Pa | N₂ | 1200Pa |
| 18 | 7 | 0.7 | 1340 | Vacuum | 10 | 1575 | He | 1000Pa | 1.5 | He | 1000Pa | N₂ | 1000Pa |

| | | | | | | | | | | | | | |
|---|---|---|---|---|---|---|---|---|---|---|---|---|---|
| The samples marked "*" are out of the scope of the present invention. | | | | | | | | | | | | | |

**[Table 5]**

| Sample No. | Interior | | | | | | | Mn ratio (% by mass) | Surface region | | | | |
|---|---|---|---|---|---|---|---|---|---|---|---|---|---|
| | dᵢ¹⁾ | aᵢ²⁾ | bᵢ³⁾ | bᵢ/aᵢ | Aᵢ⁴⁾ | Bᵢ⁵⁾ | Bᵢ/Aᵢ | | bₛ⁶⁾ | bₛ/bᵢ | Bₛ⁷⁾ | cₛ/cᵢ⁸⁾ | Thickness (*µ*m) |
| 12 | 0.45 | 0.35 | 1.25 | 3.57 | 27 | 73 | 2.70 | 0.24 | 1.75 | 1.40 | 94 | 0.05 | 2.1 |
| 13 | 0.52 | 0.26 | 0.85 | 3.27 | 40 | 60 | 1.50 | 0.15 | 1.30 | 1.53 | 92 | 0.03 | 1.2 |
| 14 | 0.43 | 0.41 | 1.45 | 3.54 | 23 | 77 | 3.35 | 0.25 | 2.10 | 1.45 | 93 | 0.07 | 4.2 |
| 15 | 0.50 | 0.21 | 1.05 | 5.00 | 37 | 63 | 1.70 | 0.20 | 1.78 | 1.70 | 95 | 0.06 | 3 |
| 16 | 0.43 | 0.20 | 0.95 | 4.75 | 35 | 65 | 1.86 | 0.38 | 1.57 | 1.65 | 94 | 0.04 | 2.8 |
| 17 | 0.45 | 0.35 | 1.26 | 3.60 | 27 | 73 | 2.70 | 0.17 | 1.95 | 1.55 | 91 | 0.08 | 4.5 |
| 18 | 0.39 | 0.51 | 1.80 | 3.53 | 17 | 83 | 4.88 | 0.14 | 2.35 | 1.31 | 92 | 0.02 | 2 |

| | | | | | | | | | | | | | |
|---|---|---|---|---|---|---|---|---|---|---|---|---|---|
| The samples marked "*" are out of the scope of the present invention. 1) dᵢ: Average particle diameter (*µ*m) of whole hard phase in interior 2) a_{i:} Average particle diameter (*µ*m) of first hard phase in interior 3) bᵢ: Average particle diameter (*µ*m) of second hard phase in interior 4) Aᵢ: Percentage of area (% by area) of first hard phase in interior 5) Bᵢ: Percentage of area (% by area) of second hard phase in interior 6) bₛ: Average particle diameter (*µ*m) of second hard phase in surface region 7) Bₛ: Percentage of area (% by area) of second hard phase in surface region 8) cₛ/cᵢ: Content ratio cₛ of binder phase in surface region / content ratio cᵢ of binder phase in interior | | | | | | | | | | | | | |

**[Table 6]**

| Sample No. | Content percentage of N in surface region of cermets (Surface region / interior) | Coating layer Film thicknesses (*µ*m) are shown in parentheses. | Cutting performance¹⁾ |
|---|---|---|---|
| 12 | 1.9 | TiCN(3.5)+Al₂O₃(4)+TiN(0.5) | 80 |
| 13 | 2 | TiCN(4)+Al₂O₃(2) | 71 |
| 14 | 2.3 | TiAlN(3) | 65 |
| 15 | 1.8 | TiCN(3.5)+Al₂O₃(4)+TiN(0.5) | 85 |
| 16 | 1.7 | TiCN(4)+Al₂O₃(2) | 74 |
| 17 | 1.5 | Al₂O₃(4) | 68 |
| 18 | 1.2 | TiCN(3) | 63 |

| | | | |
|---|---|---|---|
| The samples marked "*" are out of the scope of the present invention. 1) Cutting performance: Time (min) elapsed until amount of wear reached 0.2mm | | | |

It will be noted from Tables 4 to 6 that in each of Samples Nos. 12 to 18, the surface region having a higher content of N than that in the interior thereof was formed, and the throw-away tip with the coating layer formed thereon exhibited excellent wear resistance and had satisfactory wear resistance.

### Example 3

The cermet substrates of Samples Nos. 19 to 31 were obtained under the same conditions as Example 1, except for the material compositions in Table 7 and the sintering conditions in Table 8.

**[Table 7]**

| Sample No. | Material composition¹⁾ | | | | | | | | | | | |
|---|---|---|---|---|---|---|---|---|---|---|---|---|
| | TiCN | WC | TiN | TaC | MoC | NbC | ZrC | VC | Ni | Co | Ni/(Co+Ni) | MnCO₃ |
| 19 | 55 | 18 | 5 | 0 | 0 | 10 | 1 | 1 | 2 | 8 | 0.20 | 3 |
| 20 | 50 | 15 | 10 | 2 | 0 | 12 | 1 | 1 | 2 | 7 | 0.22 | 3 |
| 21 | 63 | 18 | 3 | 1 | 1 | 3 | 1 | 1 | 4 | 5 | 0.44 | 2 |
| 22 | 50 | 18 | 11 | 0 | 0 | 9 | 0 | 2 | 2 | 8 | 0.20 | 4 |
| 23 | 48 | 18 | 10 | 4 | 1 | 8 | 1 | 2 | 1 | 7 | 0.13 | 2 |
| 24 | 48 | 15 | 13 | 0 | 4 | 10 | 1 | 1 | 3 | 5 | 0.38 | 3 |
| 25 | 60 | 20 | 10 | 1 | 0 | 1 | 1 | 1 | 4 | 2 | 0.67 | 4 |
| * 26 | 51 | 10 | 18 | 5 | 0 | 0 | 2 | 2 | 4 | 8 | 0.33 | 3 |
| * 27 | 50 | 5 | 17 | 3 | 1 | 12 | 3 | 0 | 4 | 5 | 0.44 | 3 |
| * 28 | 52 | 12 | 9 | 1 | 5 | 10 | 1 | 0 | 7 | 3 | 0.70 | 0 |
| * 29 | 49 | 10 | 14 | 0 | 5 | 10 | 1 | 1 | 3 | 7 | 0.30 | 3 |
| * 30 | 44 | 18 | 12 | 0 | 5 | 10 | 1 | 0 | 6 | 4 | 0.60 | 3 |
| * 31 | 52 | 10 | 10 | 1 | 5 | 10 | 1 | 1 | 0 | 10 | 0.00 | 0 |

| | | | | | | | | | | | | |
|---|---|---|---|---|---|---|---|---|---|---|---|---|
| The samples marked "*" are out of the scope of the present invention. 1) Material composition: The unit of materials other than MnCO₃ is "% by mass." MnCO3 is represented in "parts by mass" to 100 parts by mass of the total amount of the other materials. | | | | | | | | | | | | |

**[Table 8]**

| Sample No. | Step (b) | | Step (c)(d) | | | | Step (e) |
|---|---|---|---|---|---|---|---|
| | Temperature T₁ (°C) | Temperature rising rate a (°C/min) | Step (c) gas pressure (Pa) | Temperature T₂ (°C) | Step (d) gas pressure (Pa) | Time (hr) | Gas pressure (MPa) |
| 19 | 1350 | 1 | 800 | 1525 | 800 | 1 | 0.2 |
| 20 | 1380 | 0.6 | 800 | 1575 | 500 | 1 | 0.1 |
| 21 | 1330 | 0.1 | 500 | 1525 | 1000 | 1 | 0.1 |
| 22 | 1350 | 0.1 | 2000 | 1575 | 1000 | 0.5 | 0.1 |
| 23 | 1330 | 2 | 500 | 1575 | 800 | 2 | 0.1 |
| 24 | 1300 | 0.6 | 500 | 1575 | 500 | 1.5 | 0.3 |
| 25 | 1400 | 1 | 9 × 10⁵ | 1600 | 9 × 10⁶ | 1.5 | 0.6 |
| * 26 | 1450 | 3 | 800 | 1550 | 800 | 1 | 0.1 |
| * 27 | 1150 | 1 | 800 | 1550 | 500 | 1 | 0.1 |
| * 28 | 1350 | 1 | 500 | 1550 | 500 | 1 | 0.1 |
| * 29 | 1350 | 1 | 500 | 1575 | Vacuum | 1 | 0.1 |
| * 30 | 1350 | 1 | 3000 | 1525 | 800 | 1 | Vacuum |
| * 31 | 1350 | 1 | 3000 | 1525 | 800 | 1 | 0.1 |

| | | | | | | | |
|---|---|---|---|---|---|---|---|
| The samples marked "*" are out of the scope of the present invention. | | | | | | | |

Each of the obtained cermets was subjected to a scanning electron microscope (SEM) observation, and an image analysis was performed using commercially available image analysis software onto arbitrary five points in the surface and the interior thereof, respectively, at a region of 8 µm x 8 µm in a photograph taken at 10000 magnification. Then, it was confirmed whether or not the surface region existed and the binder phase-rich region existed by observing the existing states of the hard phase, and the structure states in the interior and the surface. Subsequently, the average particle diameter of each of these regions was measured, and the ratio thereof was calculated. Further, the content ratio of the Mn ingredient in the cermet substrate of each sample was determined by ICP analysis. The results were shown in Table 9.

**[Table 9]**

| Sample No. | Interior structure | | | Binder phase-rich region | | | Surface region | | |
|---|---|---|---|---|---|---|---|---|---|
| | Average particle diameter of hard phase (*µ*m) | Mn ratio (% by mass) | Content ratio B of binder phase (% by mass) | Content ratio A of binder phase (% by mass) | A/B | Thickness (*µ*m) | Ratio of binder phase (% by mass) | Thickness (*µ*m) | Nb ratio (% by mass) |
| 19 | 0.7 | 0.2 | 10 | 18 | 1.5 | 2.5 | 1.5 | 2.1 | 15 |
| 20 | 0.8 | 0.1 | 9 | 9.9 | 1.3 | 4.7 | 1.2 | 1.5 | 21.6 |
| 21 | 0.6 | 0.2 | 9 | 9.9 | 1.2 | 3.9 | 1.7 | 2.3 | 7.2 |
| 22 | 1 | 0.3 | 10 | 13 | 1.7 | 2.3 | 0.9 | 1.7 | 16.2 |
| 23 | 0.9 | 0.4 | 8 | 12 | 1.8 | 1.8 | 2.5 | 5 | 17.6 |
| 24 | 1.5 | 0.4 | 8 | 16 | 2 | 2.1 | 2.8 | 2.7 | 21 |
| 25 | 2 | 0.5 | 6 | 6.6 | 2.1 | 3.5 | 3 | 1.5 | 2.8 |
| * 26 | 0.8 | 0.1 | 12 | 35 | 2.9 | 7.9 | - | | |
| * 27 | 0.8 | 1.5 | 9 | 9.9 | 1.1 | 3.6 | 5.4 | 8.3 | 21.6 |
| * 28 | 0.8 | <0.05 | 10 | - | | | - | | |
| * 29 | 0.8 | 0.1 | 10 | - | | | - | | |
| * 30 | 0.8 | 2.2 | 10 | 2.3 | 0.2 | 1.2 | - | | |
| * 31 | 0.8 | <0.05 | 10 | - | | | - | | |

| | | | | | | | | | |
|---|---|---|---|---|---|---|---|---|---|
| The samples marked "*" are out of the scope of the present invention. | | | | | | | | | |

Next, the coating layers having the structures shown in Table 11 were formed on the above cermet substrates by CVD method under the film forming conditions shown in Table 10, respectively. As shown in Table 11, in the scanning electron microscopic observations of Samples Nos. 19 to 22 and 24 in which a TiCN layer having a film thickness of not less than 2 µm was formed, it was confirmed that these samples were composed of the columnar crystal having an average crystal width of 0.1 to 1 µm extending vertically with respect to the surface of the cermet substrate, as shown in the photograph of Sample No. 24 in Figs. 2(a) and 2(b). In each of their respective X-ray diffraction measurements, the peak of (422) plane was the strongest.

**[Table 10]**

| Coating layer | Mixed gas composition (% by volume) | Mixed gas flow rate (ℓ/min) | Film forming temperature (°C) | Pressure (kPa) |
|---|---|---|---|---|
| TiN | TiCl₄:0.5, N₂:33, H₂:The rest | 80 | 900 | 16 |
| TiCN | TiCl₄:1.0, N₂:30, CH₃CN:0.4, H₂:The rest | 70 | 820 | 9 |
| TiCNO | TiCl₄:0.7, CH₄:4, N₂:5, CO₂:1.0, H₂:The rest | 35 | 1010 | 10 |
| TiNO | TiCl₄:0.7, CH₄:4, N₂:5, CO₂:1.1, H₂:The rest | 35 | 1010 | 10 |
| TiC | TiCl₄:1.0, CH4:6, H2:The rest | 65 | 1000 | 10 |
| Al₂O₃ | AlCl₃:15, HCl:2, CO₂:4, H₂S:0.01, H₂:The rest | 35 | 1005 | 6 |
| ZrN | ZrCl₄:2.0, N₂:20, H₂:The rest | 70 | 1010 | 16 |

Next, the obtained cutting tools made of the cermets were subjected to cutting tests under the following cutting conditions. The results were shown in Table 11.

**<Wear resistance test>**

| | |
|---|---|
| Work material: | SCM435 |
| Cutting speed: | 200m/min |
| Feed rate: | 0.20mm/rev |
| Depth of cut: | 1.0mm |
| Cutting state: | Wet (using water-soluble cutting fluid) |
| Evaluation method: | Time (min) elapsed until the amount of wear reached 0.2mm |

**<Fracture resistance test>**

| | |
|---|---|
| Work material: | SCM440 |
| Cutting speed: | 100m/min |
| Feed rate: | 0.05mm/rev (increased by 0.05mm/rev at 10 seconds intervals, a maximum of 0.50mm/rev) |

| | |
|---|---|
| Depth of cut: | 1.5mm |
| Cutting state: | Dry |
| Evaluation method: | Time measured until the cutting edge was fractured (a maximum of 100 seconds) |

**[Table 11]**

| Sample No. | Structure of coating layers Film thicknesses (*µ*m) are shown in parentheses. | | | | | | Wear resistance (Cutting time) (min) | Fracture resistance (Cutting time) (sec) |
|---|---|---|---|---|---|---|---|---|
| | First layer | Second layer | Third layer | Fourth layer | Fifth layer | Nb diffusion¹⁾ | | |
| 19 | TiCN (4) | TiCNO (0.5) | Al₂O₃ (2) | TiN (0.5) | - | Yes | 88 | 100 |
| 20 | TiCN (4) | TiCNO (0.2) | Al₂O₃ (2) | - | - | Yes | 82 | 94 |
| 21 | TiCN (5) | TiCNO (0.5) | Al₂O₃ (2) | ZrN (1) | - | Yes | 76 | 88 |
| 22 | TiN (0.5) | TiCN (4) | TiCNO (0.5) | Al₂O₃ (3) | TiN (0.5) | Yes | 69 | 85 |
| 23 | TiC (3) | Al₂O₃ (2) | TiN (0.5) | - | - | Yes | 68 | 84 |
| 24 | TiCN (3.5) | - | - | - | - | Yes | 71 | 79 |
| 25 | Al₂O₃ (4) | - | - | - | - | No | 73 | 73 |
| * 26 | TiCN (4) | - | - | - | - | No | 38 | 66 |
| * 27 | TiCN (4) | TiCNO (0.5) | Al₂O₃ (3) | TiN (0.5) | - | Yes | 46 | 43 |
| * 28 | TiCN (4) | TiCNO (0.5) | Al₂O₃ (3) | TiN (0.5) | - | No | 36 | 48 |
| * 29 | TiCN (4) | TiCNO (0.5) | Al₂O₃ (2) | TiN (0.5) | - | No | 43 | 36 |
| * 30 | TiN (1) | TiCN (4) | TiCNO (0.5) | Al₂O₃ (2) | TiN (0.5) | Yes | 48 | 65 |
| * 31 | TiN (0.5) | TiCN (5) | TiCNO (0.1) | Al₂O₃ (2) | TiN (0.5) | No | 44 | 25 |

| | | | | | | | | |
|---|---|---|---|---|---|---|---|---|
| The samples marked "*" are out of the scope of the present invention. 1) Nb diffusion: "Yes" indicates that the ratio of a content ratio of Nb in the region extending 0.5 *µ*m from the surface of the cermet substrate to a content ratio of Nb in the surface of the cermet substrate, in the coating layer, is 10% or more. "No" indicates that the ratio of a content ratio of Nb in the region extending 0.5 *µ*m from the surface of the cermet substrate to a content ratio of Nb in the surface of the cermet substrate, in the coating layer, is less than 10%. | | | | | | | | |

The followings will be noted from Tables 7 to 11. That is, in Sample No. 31 in which neither Ni nor Mn was added and the content of Mn was less than 0.1% by mass, a large amount of the binder phase was dispersed into the coating layer to thereby deteriorate the hardness of the coating layer, and the sintering properties of the cermet substrate was poor, thus being susceptible to chipping. In Sample No. 28 in which Mn was not added and the content of Mn was less than 0.1% by mass, the surface region was not formed and needle-shaped abnormal particles were grown in the coating layer, thus causing severe wear and fracture. In Sample No. 26 in which the sintering temperature T₁ in the step (b) was higher than 1380°C and the temperature rising rate r₁ was higher than 2°C/min in the temperature range from 1200°C to 1300-1380°C, and in Sample No. 29 in which the sintering atmosphere in the step (e) was under vacuum, and in Sample No. 30 in which the sintering atmosphere in the step (e) was under vacuum, the surface region was not formed, and needle-shaped abnormal particles were grown in the coating layer, thus deteriorating wear resistance and fracture resistance. In Sample No. 27 in which the sintering temperature T₁ in the step (b) was below 1300°C, exceeding 3% by mass of Mn remained in the cermet substrate after sintering, thus deteriorating wear resistance.

On the contrary, all Samples Nos. 19 to 25, which were the cermets having the structures within the scope of the invention, exhibited excellent wear resistance and satisfactory wear resistance, thereby achieving a long tool life.

### Explanation of marks

### BRIEF DESCRIPTION OF DRAWINGS

Fig. 1 is a scanning electron microscope (SEM) photograph showing an example of the Ti-based cermet of the invention, specifically a cross-section of important parts including a surface region thereof;
Figs. 2(a) and 2(b) are scanning electron microscope (SEM) photographs showing an example of the coated cermet of the invention, specifically cross-sections of important parts including a surface region thereof, respectively; and
Figs. 3(a) and 3(b) are schematic diagrams of an example of the cutting tool of the invention.

### EXPLANATION OF REFERENCE

- 1: Cermet(Ti-based cermet)
- 2: Hard phase
2a First hard phase
2b Second hard phase
- 3: Binder phase
- 5: Surface region
- 8: Binder phase-rich region
- 10: Coated cermet
- 12: Substrate
- 13: Coating layer
- 20: Cutting tool
- 21: Rake face
- 22: Flank face
- 23: Cutting edge
- 24: Breaker
- 25: Recessed part
- 26: Screw hole

## Claims

1. A Ti-based cermet (1) comprising at least one kind of element selected from Co and Ni; one or more kinds of substances selected from carbides, nitrides, and carbonitrides of one or more kinds of metals selected from Group 4, Group 5, and Group 6 metals of the periodic table,
composed mainly of Ti; and 0.1 to 0.5% by mass of Mn, wherein in a scanning electron microscope (SEM) photograph of an arbitrary cross-section of the Ti-based cermet, a surface region (5) of a thickness of 0.5 to 5 µm is formed in which a hard phase (2) whose interior comprises a first hard phase (2a) and a second hard phase (2b), and a binder phase (3) composed mainly of at least one kind of element selected from Co and Ni are observed, and the first hard phase (2a) has a higher content ratio of a light element than the second hard phase (2b), and in the surface region the second hard phase (2b) is observed in a percentage of not less than 90%.

2. The Ti-based cermet (1) according to claim 1, wherein Nb is dissolved in the second hard phase (2b) to form a solid solution, and the proportion of Nb dissolved in the second hard phase (2b) to form solid solution in the surface region (5) is larger than the proportion of Nb dissolved in the second hard phase (2b) to form solid solution in the interior.

3. A method of manufacturing a Ti-based cermet (1) comprising the steps of:
forming a mixed powder as a mixture of TiCN powder; at least one kind of powder selected from carbide powder, nitride powder and carbonitride powder each containing one or more kinds of elements selected from W, Mo, Ta, V, Zr and Nb; at least one kind of powder selected from Co and Ni; and a total amount of 0.2 to 3.0% by mass in terms of Mn of a metal Mn powder or an Mn compound powder; and
sintering the mixed powder under the following conditions:
(a) temperature is increased under vacuum from room temperature to 1200°C;
(b) the temperature is increased under vacuum at a temperature rising rate of 0.1 to 2°C/min from 1200°C to a sintering temperature T₁ of 1330°C to 1380°C;
(c) the temperature is increased at a temperature rising rate of 4 to 15°C/min from the sintering temperature T₁ to a sintering temperature T₂ of 1450 to 1600°C in an inert gas atmosphere of 30 to 2000 Pa;
(d) the sintering temperature T₂ is retained in the inert gas atmosphere of 30 to 2000 Pa for 0.5 to 2 hours; and
(e) the temperature is decreased in a vacuum or an inert gas atmosphere.

4. A coated cermet (10) comprising a substrate (12) comprising the Ti-based cermet (1) according to claim 1 or 2, and a coating layer (13) coating a surface of the substrate (12), wherein the content ratio of the binder phase (3) in the surface region (5) of the substrate (12) is not more than 3% by mass, and the coating layer (13) is formed by chemical vapor deposition.

5. The coated cermet (10) according to claim 4, wherein a binder phase-rich region (8) exists in a region extending 1 to 10 µm from immediately below the surface region (5), at 1.1 to 2.0 in terms of a ratio (A/B) of a content ratio A of the binder phase (3) to a content ratio B of the binder phase (3) in the interior of the substrate (12).

6. The coated cermet (10) according to claim 4 or 5, wherein the content ratio of Ni in the interior of the substrate (12) is 0.1 to 0.5 in terms of Ni/(Ni+Co) ratio.

7. The coated cermet (10) according to any one of claims 4 to 6, wherein the content percentage of N in the surface region (5) is larger than that of the interior of a sintered body.

8. The coated cermet (10) according to any one of claims 4 to 7, wherein the coating layer (13) is composed of a columnar crystal extending vertically with respect to the surface of the substrate (12), and the columnar crystal has an average crystal width of 0.1 to 1 µm.

9. The coated cermet (10) according to claim 8, wherein the columnar crystal is TiCN.

10. The coated cermet (10) according to claim 9, wherein the coating layer (13) has its strongest peak in (422) plane in an X-ray diffraction measurement.

11. A cutting tool (20) comprising the Ti-based cermet (1) according to claim 1 or 2, or the coated cermet (10) according to any one of claims 4 to 10, wherein a cutting edge (23) is formed along a cross ridge part between a rake face (21) and a flank face (22).

12. The cutting tool (20) according to claim 11, wherein in the residual stress exerted in a σ11 direction (namely, a direction to connect between the center of the rake face (21) and the center of the cutting edge (23) nearmost a measured point) measured in the rake face (21) by 2D method, the second hard phase (2b) is subjected to compressive stress of not less than 150 MPa (σ11 ≤ -150 MPa).

## Patentansprüche

1. Ein Ti-basiertes Cermet(1), aufweisend mindestens eine Art von Element, das aus Co und Ni ausgewählt ist, eine oder mehrere Arten von Stoffen, die aus Carbiden, Nitriden und Carbonitriden einer oder mehrerer Arten von Metallen ausgewählt sind, die aus Metallen der Gruppe 4, der Gruppe 5 und der Gruppe 6 des Periodensystems ausgewählt sind, zusammengesetzt hauptsächlich aus Ti, und 0,1 bis 0,5 Masse-% Mn, wobei in einer Rasterelektronenmikroskop- (REM) - Fotografie eines beliebigen Querschnitts des Ti-basierten Cermets ein Oberflächenbereich (5) mit einer Dicke von 0,5 bis 5 µm ausgebildet ist, in dem eine Hartphase (2), deren Inneres eine erste Hartphase (2a) und eine zweite Hartphase (2b) aufweist, und eine Bindemittelphase (3), die hauptsächlich aus mindestens einer Art von Element zusammengesetzt ist, das aus Co und Ni ausgewählt ist, beobachtet werden, und die erste Hartphase (2a) einen höheren Gehalt eines leichten Elements als die zweite Hartphase (2b) aufweist, und im Oberflächenbereich die zweite Hartphase (2b) in einem Prozentanteil von nicht weniger als 90% beobachtet wird.

2. Das Ti-basierte Cermet (1) gemäß Anspruch 1, wobei Nb in der zweiten Hartphase (2b) gelöst ist, um eine feste Lösung zu bilden, und der Anteil von Nb, das in der zweiten Hartphase (2b) gelöst ist, um eine feste Lösung zu bilden, im Oberflächenbereich (5) größer als der Anteil von Nb, das in der zweiten Hartphase (2b) gelöst ist, um eine feste Lösung zu bilden, im Inneren ist.

3. Ein Verfahren zum Herstellen eines Ti-basierten Cermets (1), aufweisend die folgenden Schritte:
Bilden eines Mischpulvers als eine Mischung aus TiCN-Pulver, mindestens einer Art von Pulver ausgewählt aus Carbidpulver, Nitridpulver und Carbonitridpulver, die jeweils eine oder mehrere Arten von Elementen enthalten, die aus W, Mo, Ta, V, Zr und Nb ausgewählt sind, mindestens einer Art von Pulver ausgewählt aus Co und Ni, und einer Gesamtmenge, bezogen auf Mn, eines Metall-Mn-Pulvers oder eines Mn-Verbindung-Pulvers von 0,2 bis 3,0 Masse-%, und
Sintern des Mischpulvers unter den folgenden Bedingungen:
(a) die Temperatur wird unter Vakuum von Raumtemperatur auf 1200°C erhöht,
(b) die Temperatur wird unter Vakuum mit einer Temperaturanstiegsrate von 0,1 bis 2°C/min von 1200°C auf eine Sintertemperatur T₁ von 1330°C bis 1380°C erhöht,
(c) die Temperatur wird mit einer Temperaturanstiegsrate von 4 bis 15°C/min in einer Inertgasatmosphäre von 30 bis 2000 Pa von der Sintertemperatur T₁ auf eine Sintertemperatur T₂ von 1450 bis 1600°C erhöht,
(d) die Sintertemperatur T₂ wird für 0,5 bis 2 Stunden in der Inertgasatmosphäre von 30 bis 2000 Pa gehalten, und
e) die Temperatur wird in einem Vakuum oder einer Inertgasatmosphäre gesenkt.

4. Ein beschichtetes Cermet (10), aufweisend ein Substrat (12), welches das Ti-basierte Cermet (1) gemäß Anspruch 1 oder 2 aufweist, und eine Beschichtungsschicht (13), die eine Fläche des Substrats (12) beschichtet, wobei der Gehalt der Bindemittelphase (3) im Oberflächenbereich (5) des Substrats (12) nicht mehr als 3 Masse-% beträgt und die Beschichtungsschicht (13) durch chemische Gasphasenabscheidung gebildet ist.

5. Das beschichtete Cermet (10) gemäß Anspruch 4, wobei in einem Bereich, der sich 1 bis 10 µm von unmittelbar unterhalb des Oberflächenbereichs (5) erstreckt, ein bindemittelphasenreicher Bereich (8) mit 1,1 bis 2,0 bezogen auf ein Verhältnis (A/B) eines Gehalts A der Bindemittelphase (3) zu einem Gehalt B der Bindemittelphase (3) im Inneren des Substrats (12) existiert.

6. Das beschichtete Cermet (10) gemäß Anspruch 4 oder 5, wobei der Gehalt von Ni im Inneren des Substrats (12) bezogen auf das Verhältnis Ni/(Ni+Co) 0,1 bis 0,5 beträgt.

7. Das beschichtete Cermet (10) gemäß irgendeinem der Ansprüche 4 bis 6, wobei der Gehalt von N im Oberflächenbereich (5) größer als der des Inneren eines Sinterkörpers ist.

8. Das beschichtete Cermet (10) gemäß irgendeinem der Ansprüche 4 bis 7, wobei die Beschichtungsschicht (13) aus einem säulenförmigen Kristall zusammengesetzt ist, der sich in Bezug auf die Oberfläche des Substrats (12) vertikal erstreckt, und der säulenförmige Kristall eine durchschnittliche Kristallbreite von 0,1 bis 1 µm hat.

9. Das beschichtete Cermet (10) gemäß Anspruch 8, wobei der säulenförmige Kristall TiCN ist.

10. Das beschichtete Cermet (10) gemäß Anspruch 9, wobei die Beschichtungsschicht (13) bei einer Röntgenbeugungsmessung ihren stärksten Peak in der (422)-Ebene hat.

11. Ein Schneidwerkzeug (20), aufweisend das Ti-basierte Cermet (1) gemäß Anspruch 1 oder 2 oder das beschichtete Cermet (10) gemäß irgendeinem der Ansprüche 4 bis 10, wobei eine Schneidkante (23) entlang eines Quergratteils zwischen einer Spanfläche (21) und einer Flankenfläche (22) ausgebildet ist.

12. Das Schneidwerkzeug (20) gemäß Anspruch 11, wobei bei der Eigenspannung, die in einer σ11-Richtung (nämlich einer Richtung zum Verbinden zwischen der Mitte der Spanfläche (21) und der Mitte der Schneidkante (23) am nächsten bei einem gemessenen Punkt) ausgeübt wird, die mittels eines 2D-Verfahrens in der Spanfläche (21) gemessen wird, die zweite Hartphase (2b) einer Druckspannung von nicht weniger als 150 MPa ausgesetzt wird (σ11 ≤ -150 MPa).

## Revendications

1. Un cermet à base de Ti (1) comprenant au moins un type d'élément choisi parmi Co et Ni ; un ou plusieurs types de substances choisies parmi les carbures, les nitrures et les carbonitrures d'un ou plusieurs types de métaux choisis parmi les métaux du groupe 4, du groupe 5 et du groupe 6 du tableau périodique, composés principalement de Ti ; et 0,1 à 0,5% en masse de Mn, où dans une photographie au microscope électronique à balayage (MEB) d'une section transversale arbitraire du cermet à base de Ti, une région de surface (5) d'une épaisseur de 0,5 à 5 µm est formée, dans laquelle une phase dure (2) dont l'intérieur comprend une première phase dure (2a) et une deuxième phase dure (2b), et une phase liante (3) composée principalement d'au moins un type d'élément choisi parmi Co et Ni sont observées, et la première phase dure (2a) a une teneur en un élément léger supérieure à la deuxième phase dure (2b), et dans la zone de surface la deuxième phase dure (2b) est observée en pourcentage non inférieur à 90%.

2. Le cermet à base de Ti (1) selon la revendication 1, dans lequel Nb est dissous dans la deuxième phase dure (2b) pour former une solution solide, et la proportion de Nb dissous dans la deuxième phase dure (2b) pour former une solution solide dans la région de surface (5) est supérieure à la proportion de Nb dissous dans la deuxième phase dure (2b) pour former une solution solide dans l'intérieur.

3. Un procédé de fabrication d'un cermet à base de Ti (1) comprenant les étapes suivantes consistant à :
former une poudre mélangée sous forme d'un mélange de poudre de TiCN, d'au moins un type de poudre choisie parmi la poudre de carbure, la poudre de nitrure et la poudre de carbonitrure, contenant chacune un ou plusieurs types d'éléments choisis parmi W, Mo, Ta, V, Zr et Nb, d'au moins un type de poudre choisie parmi Co et Ni, et d'une quantité totale, en termes de Mn, d'une poudre Mn métallique ou d'une poudre de composé de Mn de 0,2 à 3,0% en masse, et
fritter la poudre mélangée dans les conditions suivantes :
a) la température est augmentée sous vide de la température ambiante à 1200 °C ;
(b) la température est augmentée sous vide à une vitesse de montée en température de 0,1 à 2°C/min de 1200°C à une température de frittage T₁ de 1330°C à 1380°C ;
(c) la température est augmentée à une vitesse de montée en température de 4 à 15°C/min de la température de frittage T₁ à une température de frittage T₂ de 1450 à 1600°C dans une atmosphère de gaz inerte de 30 à 2000 Pa ;
d) la température de frittage T₂ est maintenue dans l'atmosphère de gaz inerte de 30 à 2000 Pa pendant 0,5 à 2 heures ; et
e) la température est abaissée dans une atmosphère de vide ou de gaz inerte.

4. Un cermet revêtu (10) comprenant un substrat (12) comprenant le cermet à base de Ti (1) selon la revendication 1 ou 2, et une couche de revêtement (13) recouvrant une surface du substrat (12), dans lequel la teneur de la phase liante (3) dans la région de surface (5) du substrat (12) n'est pas supérieur à 3% en masse et la couche de revêtement (13) est formée par dépôt chimique en phase vapeur.

5. Le cermet revêtu (10) selon la revendication 4, dans lequel une région riche en phase liante (8) existe dans une région s'étendant de 1 à 10 µm depuis immédiatement au-dessous de la région de surface (5), à 1,1 à 2,0 en termes de rapport (A/B) d'une teneur A de la phase liante (3) sur une teneur B de la phase liante (3) à l'intérieur du substrat (12) .

6. Le cermet revêtu (10) selon la revendication 4 ou 5, dans lequel la teneur en Ni à l'intérieur du substrat (12) est de 0,1 à 0,5 en termes de rapport Ni/(Ni+Co).

7. Le cermet revêtu (10) selon l'une quelconque des revendications 4 à 6, dans lequel la teneur en N dans la région de surface (5) est supérieure à celle de l'intérieur d'un corps fritté.

8. Le cermet revêtu (10) selon l'une quelconque des revendications 4 à 7, dans lequel la couche de revêtement (13) est composée d'un cristal en forme de colonne s'étendant verticalement par rapport à la surface du substrat (12), et le cristal en forme de colonne a une largeur de cristal moyenne de 0,1 à 1 µm.

9. Le cermet revêtu (10) selon la revendication 8, dans lequel le cristal en colonne est du TiCN.

10. Le cermet revêtu (10) selon la revendication 9, dans lequel la couche de revêtement (13) a son pic le plus fort dans le plan (422) dans une mesure de diffraction des rayons X.

11. Un outil de coupe (20) comprenant le cermet à base de Ti (1) selon la revendication 1 ou 2, ou le cermet revêtu (10) selon l'une quelconque des revendications 4 à 10, dans lequel une arête de coupe (23) est formée le long d'une partie de nervure transversale entre une face de coupe (21) et une face de flanc (22).

12. L'outil de coupe (20) selon la revendication 11, dans lequel, dans la contrainte résiduelle exercée dans une direction σ11 (à savoir, une direction pour relier entre le centre de la face de coupe (21) et le centre de l'arête de coupe (23) le plus près un point mesuré) mesurée dans la face de coupe (21) par procédé 2D, la deuxième phase dure (2b) est soumise à une contrainte en compression non inférieure à 150 MPa (σ11 ≤ -150 MPa).
